

July 19, 1949.

R. E. CHURCHWARD ET AL

2,476,284

COBALT SOLUTION PURIFICATION

Filed Jan. 1, 1945



*Fig. 1*



*Fig. 2*

Inventors.

RUTH E. CHURCHWARD

FRANCIS K. SHELTON

By *Roy E. Shuckley Jr.*  
Attorney.

## UNITED STATES PATENT OFFICE

2,476,284

## COBALT SOLUTION PURIFICATION

Ruth E. Churchward and Francis K. Shelton,  
Boulder City, Nev.

Application January 1, 1945, Serial No. 570,936

2 Claims. (Cl. 23—50)

(Granted under the act of March 3, 1883, as  
amended April 30, 1928; 370 O. G. 757)

1

The invention described herein may be manufactured and used by or for the Government of the United States for governmental purposes without the payment to us of any royalty thereon in accordance with the provisions of the act of April 30, 1928 (Ch. 460, 45 Stat. L. 467).

This invention relates to the production of purified cobalt compounds, and more particularly to the production of a cobalt compound of sufficient purity to be suitable for metallic cobalt electrowinning purposes.

In the production of metallic cobalt by electrolysis from a suitable solution, such as for example one containing cobalt sulfate, boric acid and sodium fluoride, it is important to remove as completely as possible any impurities interfering with the rapid and smooth plating out of the cobalt metal. Certain harmful impurities occur in relatively large amounts in cobalt solutions prepared by usual methods, suitably by extracting cobalt ore concentrates with acids. Among such impurities are zinc, copper, iron, cadmium, mercury, arsenic, and antimony. Other harmful impurities which are present or may occasionally be present are gallium, thallium, bismuth, palladium, ruthenium, osmium and indium. These latter substances may be present in such small amounts as to defy chemical detection, but nevertheless interfere with a satisfactory cobalt electrodeposition.

It is accordingly an object of this invention to prepare a purified cobalt compound suitable for metallic cobalt electrowinning purposes and a further object is the purification of contaminated cobalt electrolytes. Many other objects and advantages will be apparent or will appear hereinafter as the ensuing description proceeds.

The foregoing and other objects are accomplished in accordance with this invention wherein an acidic cobalt solution is treated to precipitate impurities from solution and a purified cobalt compound, suitable for electrowinning purposes, is recovered.

More specifically, according to one feature of this invention, a solution of a soluble cobalt salt under acidic conditions is treated with a soluble sulfide, and a purified cobalt compound in solution is separated from the insoluble residue precipitate. Suitable soluble cobalt salts include the salts prepared by treating a cobalt ore with an acid such as for example a strong mineral acid which may include nitric acid, hydrochloric acid and preferably sulfuric acid. For illustrative purposes, the invention will be described in con-

nection with the purification of a cobalt sulfate solution but it is not to be limited thereto.

Suitable soluble sulfides for employment in accordance with this invention include the soluble sulfides and polysulfides of the alkali metals and ammonia, examples being ammonium sulfide, potassium sulfide, and sodium sulfide. Preferably, for reasons of economy, convenience and purity of the resulting cobalt compound, hydrogen sulfide is employed as a soluble sulfide precipitating reagent.

Desirably, hydrogen sulfide is employed under an elevated superatmospheric pressure of at least ten pounds per square inch gauge, suitably between 15 and 100 pounds per square inch gauge. In general we have found a pressure of about 20 pounds per square inch gauge to be entirely satisfactory and preferable. However, the upper limit of pressure under which our sulfide treatment is carried out is limited only by the strength of the reaction equipment.

The treatment of the cobalt sulfate or other soluble cobalt salt in solution with a soluble sulfide is carried out under acidic solution conditions, and generally the solution is maintained within an acidity range between about pH 1 and pH 6, and preferably the acidity is maintained within the more restricted range of between about pH 4 and pH 5. The pH or solution acidity may be brought and maintained within the desired range by any of the customary means known to those skilled in the art, but ordinarily we prefer to incorporate cobalt oxide or carbonate to elevate the solution pH when necessary, and an innocuous mineral acid such as for example boric acid, sulfuric acid or hydrochloric acid, can be employed to lower the solution pH.

Suitable apparatus for carrying out the precipitation treatment of this invention is illustrated in the accompanying drawings in which:

Figure 1 illustrates in diagrammatic form a suitable arrangement of apparatus.

Figure 2 illustrates in diagrammatic form a somewhat simpler alternative arrangement of suitable apparatus for carrying out this invention.

In operation, and referring now to the drawings, cobalt solution to be treated is stored in a suitable container 11 and a soluble sulfide, for example hydrogen sulfide is stored in another suitable vessel 14. Cobalt solution from the container 11 passes by way of a pump 20 through a pair of inlet valves 22 and 19 into a pair of reaction vessels 12 and 13. During introduction of the cobalt solution, a pressure relief valve 17 is maintained in the open position. The cobalt

solution is allowed to enter the reaction vessels 12 and 13 until the liquid level indicator 16 shown as a sight glass indicates a suitable quantity of cobalt solution has been admitted. Thereupon, the pump 20 and the inlet valves 22 and 19, are closed and the pressure relief valve 17 is likewise closed. Hydrogen sulfide or other soluble sulfide is admitted to the reaction vessels 12 and 13, which are interconnected at their upper portions by a pipe 28 and through their lower portions by 10 a pipe system including a valve 23, a second pump 25 provided with a priming device 27 and a second valve 24. After admission of hydrogen sulfide from the storage vessel 14 through inlet valve 31 and a suitable pipe 30, the pressure upon the 15 reaction chambers 12 and 13 is elevated to a predetermined value as indicated on a suitable gauge 15 which may be 20 pounds per square inch guage. Thereupon, the valves 23 and 24 are opened, the circulating pump 25 is started, and the solution in the reaction chambers proceeds from one chamber 13 through pump 25 and the second chamber 12 and thence back to chamber 13 by way of circulating leg 28 which is optionally provided with a spray head 29 in chamber 13.

The circulation is continued until a desired degree of saturation is obtained, then thereupon the sulfide inlet valve 31 is closed, the circulating pump 25 is stopped, the vent valve 11 is opened to release excess pressure and the discharge valve 21 is opened thus draining the reaction chambers 12 and 13 into a storage and settling tank 18. The purified solution can be separated from the formed precipitate by decantation, filtration and the like in suitable apparatus not shown. Thereupon, the purified cobalt compound can be recovered from the purified solution, if desired, by crystallization, evaporation and the like. Desirably, purified solution has incorporated therein about 50 grams per liter of boric acid and 5 grams per liter of sodium fluoride to form a suitable fluoborate electrolyte for cobalt electrowinning.

An alternative arrangement of suitable apparatus as shown in Figure 2 comprises an elevated storage vessel 38 communicating with a lower reaction vessel 40 by way of pump 51, a regulating valve 50 and a pipe 49. The lower reaction vessel 40 is connected to the upper container 48 by means of the elevated pipe system 42 and 44 designed to place the pipe section 44 under a suitably elevated pressure for carrying out the treatment. Hydrogen sulfide or other soluble sulfide is admitted to the system from a suitable storage container 46 by way of an inlet valve 47 and a pump 41 which serves both to circulate the treatment liquors and to create a suitable pressure in the pipe section 44 in conjunction with the regulating valve 45. The pressure existing in the pipe section 44 is dependent upon the vertical height thereof as well as with pressure created by the pump 41 and maintained by the regulating valve 45. In operation, the pumps 41 and 51 are started, hydrogen sulfide is admitted to the system and the solution undergoing treatment proceeds from storage vessel 48 through the pump 51 and the pipe 49 into a reaction vessel 40 and thence through low pressure pipe 42 into the high pressure pipe 44 where it is treated with hydrogen sulfide admitted through the pump 41. The solution then passes through regulating valve 45 and into storage chamber 48 again. After a suitable length of treatment, the pumps may be stopped, and the treated solution allowed to settle in container 48 from which purified cobalt solution can be decanted by means not shown.

In addition to the simple treatment of the soluble cobalt compound under acidic conditions with a soluble sulfide as described above, we have found it highly desirable to carry out the sulfide treatment in the presence of a precipitate-forming amount of a normally soluble salt of a heavy metal from the group of copper and iron, then treating the resulting mixture with an innocuous oxidizing agent, and separating a purified cobalt solution from the impurity-containing residue. Desirably, this precipitation treatment can be carried out by dissolving an excess of a soluble copper compound and a soluble iron compound in a cobalt solution to be purified, then precipitating from said solution an insoluble copper compound together with impurities, and thereafter an insoluble iron compound together with further impurities. We have found that the precipitation of an insoluble copper compound from solution carries with it not only the undesired copper sulfide but also a great many impurities which cannot be determined chemically but which detrimentally affect the subsequent electrolysis of the cobalt solution and tend to yield a poor metallic cobalt deposit. Desirably, the previously sulfide treatment is carried out in the presence of at least .1 gram of a normally soluble copper compound per liter of solution and usually the sulfide treatment should be carried out in the presence of between .1 and 10 grams of a normally soluble copper compound per liter of solution. The copper compound can be added in the form of any of the normally soluble compounds of copper such as for example copper nitrate, copper formate, copper acetate, copper chloride, and preferably copper sulfate.

It has also been found, that the precipitation of an iron compound from solution also carries with it a great number of impurities which detrimentally affect subsequent electrolysis of the cobalt solution. The exact nature of the impurities cannot definitely be determined, but electrolysis of a cobalt solution before and after treatment in accordance with the iron precipitation step about 40 to be described establishes beyond question the efficacy of our iron precipitation treatment. In carrying out this precipitation we treat the solution, either before or after the sulfide treatment, with an excess of an innocuous oxidizing 45 agent in the presence of at least .1 gram of dissolved iron per liter of cobalt solution undergoing treatment. Generally, it has been found that between about .1 and 10 grams of dissolved iron per liter of solution forms a suitable amount of dissolved iron for precipitation. The dissolved iron is preferably precipitated by treatment at an acidity not more acid than pH 3.2 and at elevated solution temperature of at least about 50 to 60 degrees centigrade. The cobalt solution containing 50 a suitable quantity of dissolved iron is treated by passing atmospheric air into and through the solution until substantially all of the dissolved iron is precipitated in the form of flocculent ferric hydroxide. Other suitable oxidizing agents can 55 be employed instead of atmospheric air, examples being hydrogen peroxide, sodium perborate and similar oxidizing agents which do not detrimentally affect subsequent electrolysis of the solution. Atmospheric air is cheap and convenient 60 and constitutes a preferred innocuous oxidizing agent for employment in accordance with this invention.

While we have separately described the foregoing sulfide treatment, copper precipitation and 65 iron precipitation, we have found that these steps

are desirably combined to yield a highly purified cobalt compound which, when subjected to electrolysis in a customary electrolyte, yields a smooth, bright continuous cobalt deposit from strongly concentrated electrolytes not heretofore yielding a satisfactory deposit at elevated concentrations. For example, by first treating the cobalt solution with solution sulfide in the presence of dissolved copper as above described, then separating the precipitate, then aerating the solution in the presence of suitable quantity of dissolved iron, again separating the precipitate, and forming a cobalt electrolyte by the addition of a suitable quantity of boric acid and sodium fluoride, we can secure very satisfactory electrodepositions at concentrations as high as 30 grams per liter of dissolved cobalt or even at higher concentrations.

The following examples show how the invention may be carried out but it is not limited thereto. Parts and percentage compositions are by weight unless otherwise designated, and the temperatures given are on the centigrade scale.

#### EXAMPLE I

The cobalt was leached from 200 pounds stain-  
ierite concentrates ( $\text{CO}_2\text{O}_3 \cdot \text{H}_2\text{O}$ ), 7.01 percent cobalt, obtained from the Columbia Mine at Good-  
springs, Nevada, using 76½ gallons of water, 27  
pounds sulphuric acid and 39.7 pounds sulphur  
dioxide (to maximum efficiency—excess sulphur  
dioxide was used in the actual test). The sol-  
ution was separated from the solids and measured  
235 liters. The solution contained 97.4 percent  
of the cobalt in the concentrates. Residual cob-  
alt solutions relatively free of impurities and  
obtained as by-products on experimental work  
in the electrodeposition of cobalt were added to  
this solution to yield 278 liters of solution having  
the analysis of Table 1. To the head solution  
hydrogen-sulphide was added under atmospheric  
pressure (about 710 mm. mercury) in an inter-  
mittent manner for about three days. The pH of  
the solution was initially about 2.0 and this be-  
came gradually more acid, the lowest pH being  
1.30. However, this was periodically raised by  
the addition of calcite to above pH 1.5 whenever  
it fell below pH 1.4. In all, 7.0 pounds of hydro-  
gen sulphide were passed into the solution. The  
temperature of the solution was that found out  
of doors at Boulder City, Nevada, during the time  
of the treatment, and ranged from 10 degrees to  
25 degrees centigrade. The hydrogen sulphide  
precipitate weighed 16½ pounds and had the  
analysis given in Table 1. The hydrogen sul-  
phide precipitation was deemed complete when  
the standard colorimetric test for copper failed  
to yield a positive test for this, equivalent to one  
part per million. The solution was then further  
treated for the removal of the iron and the recov-  
ery of the cobalt.

Table 1.—Analysis of solutions and products

| Element                     | Head<br>Solution                  | Precipitate     | Pure<br>Solution |
|-----------------------------|-----------------------------------|-----------------|------------------|
| Cobalt.....                 | Grams per<br>liter<br>29.2<br>1.3 | Per cent<br>5.1 |                  |
| Nickel.....                 | 2.6                               |                 |                  |
| Iron.....                   | 5.3                               | 23.2            | Nil.             |
| Copper.....                 | 6.9                               |                 |                  |
| Manganese.....              | 0.7                               |                 |                  |
| Magnesium.....              |                                   | 7.0             |                  |
| Calcium.....                |                                   | Nil.            |                  |
| Lead.....                   |                                   | Traces          | Negative.<br>Do. |
| Bi, Cd, As, Sn, Sb, Hg..... |                                   |                 |                  |

#### EXAMPLE II

Hydrogen sulphide gas was bubbled thru 9.97  
liters impure  $\text{CoSO}_4$  solution containing 1 g. added  
5  $\text{CuSO}_4$  for one hour and twenty-five minutes.  
At the start the pH of the solution was 3.17, it  
was held between 2 and 3 by periodic additions  
of saturated soda ash solution. The sulphided  
solution was allowed to stand ½ hour and was  
then filtered by the use of filter aid. The filtrate  
10 was made into a fluoborate electrolyte for cobalt  
electrowinning by adding 50 g./l.  $\text{H}_3\text{BO}_3$  and 5  
g./l.  $\text{NaF}$ . One third of this solution was used  
as is in the cobalt electrolytic cell. The first  
15 seven hour plate was fair. Another third of the  
solution was treated as follows: The pH was  
raised to 5.95 with soda ash solution and then  
5.27 g.  $\text{FeSO}_4 \cdot 7\text{H}_2\text{O}$  were added. Finally, the sol-  
ution was warmed for 8 hours between 60 de-  
grees-70 degrees centigrade, with air bubbling  
20 thru it to oxidize the iron. It stood overnight  
and was filtered the next morning for use in the  
cell. A good seven hour plate was obtained for  
this. The pH of the final third of the electrolyte  
25 was lowered to 3.01 by adding 3 cc. concentrated  
sulphuric acid. Iron wire was then added to the  
solution, and air was bubbled through it for sev-  
eral days. Finally, the iron was removed, the  
solution oxidized, the pH adjusted to 6.0, and the  
30 solution filtered off. Upon electrolysis, an excel-  
lent plate of cobalt resulted.

#### EXAMPLE III

Two electrolytes were prepared from the solu-  
tions purified in accordance with Examples I and  
35 II by incorporating 50 grams per liter of boric  
acid and 5 grams per liter of sodium fluoride,  
and thereafter the concentrations of the two  
electrolytes were respectively adjusted to be (a)  
40 20 grams per liter and (b) 30 grams per liter  
of dissolved cobalt. When subjected to electrolysis  
in a suitable electrolytic cell employing a  
suitable current density and a suitable voltage  
the following results were secured:

Table 2.—pH time correlation

| Test   | Time<br>Treatment | pH Solution |      | Quality of Electro-<br>deposits from solutions<br>containing |              |
|--------|-------------------|-------------|------|--------------------------------------------------------------|--------------|
|        |                   | Start       | End  | 20 g./l. Co.                                                 | 30 g./l. Co. |
| 1..... | 1.0               | 1.50        | 1.87 | Good.                                                        |              |
| 2..... | 1.5               | 2.70        | 2.38 | Very good.                                                   |              |
| 3..... | 3.0               | 2.61        | 2.80 |                                                              | Good.        |
| 4..... | 3.0               | 4.22        | 3.56 |                                                              | Excellent.   |

Certain temperature correlations were made.  
Table 3 presents data secured when a given head  
sample is treated for three hours at 20 pounds  
60 per square inch gauge hydrogen sulphide pres-  
sure in three tests, and the pH of the solution  
is determined. A combination of all of the  
treated solutions yielded a good cobalt plate at  
30 g./l. cobalt concentration, for 7 hours.

Table 3.—pH temperature correlations

| Test   | Initial pH | Final pH | Temp., °C. |
|--------|------------|----------|------------|
| 1..... | 4.34       | 2.52     | 21.4       |
| 2..... | 4.34       | 1.92     | 20.5       |
| 3..... | 4.34       | 1.78     | 15.5       |

#### EXAMPLE IV

Forty liters of impure cobalt sulphate electro-  
lytes containing .1 gram per liter of copper sul-

phate and having an acidity of pH 1.5 is treated with hydrogen sulphide under a pressure of 20 pounds per square inch gauge for one hour. The solution was filtered, and had a pH 1.82. 268 grams of precipitate were removed. The pH of the solution was then raised to between 5 and 6 by addition of soda ash and 1.5 grams per liter of copperas was then added to the solution. It was then warmed to a temperature between 60 degrees and 70 degrees centigrade while a vigorous stream of air was passed through the solution and periodical additions of soda ash were added to hold the pH between 5 and 6. After 24 hours, the flocculent precipitate was removed from the solution, and at a cobalt concentration of 20 grams per liter a good plate of cobalt was produced by electrolysis, thus indicating substantial purification of the electrolyte.

## EXAMPLE V

A batch of cobalt electrolytes having a pH of 4.22 were sulphided by treatment with hydrogen sulphide under a pressure of 20 pounds per square inch for three hours. At the end of that time the solution pH was 3.56. The mixture of solution and precipitate was allowed to settle, and the solution was filtered with the aid of a suitable filter aid. The weight of the hydrogen sulphide precipitate including filter aid was 399 grams. The solution was then treated by bubbling air through it for about 12 hours and then again filtered. Then about 5 grams per liter of copperas was added to the solution, and the solution again aerated for about 12 hours and filtered. Thereupon, cobalt carbonate was precipitated from the solution by the addition of saturated soda ash solution and the precipitated cobalt carbonate was employed to make a cobalt electrolyte that is to say, it was dissolved in sulphuric acid and sufficient water to make an aqueous solution containing 30 grams per liter of cobalt then 50 grams per liter of boric acid together with 5 grams per liter of sodium fluoride was incorporated in the resulting solution. Upon electrolysis, an excellent cobalt plate, free from trees, nodules and the like was produced.

Various changes can be made in the invention as illustrated and described without departing from the spirit and scope thereof since many apparently widely differing embodiments will occur to one skilled in the art.

What is claimed is:

1. In a process for the production of a purified

cobalt solution suitable for cobalt electrowinning purposes, the steps which comprise treating an impure cobalt solution containing at least zinc as an impurity with an excess of hydrogen sulfide under an elevated pressure of at least ten pounds per square inch and at a solution pH between pH 1 and pH 6, whereby zinc is precipitated as a sulfide, and then separating a purified cobalt solution from the resulting precipitate.

2. In a process for the production of a purified cobalt solution suitable for cobalt electrowinning purposes from an impure cobalt salt solution containing at least one impurity selected from the group consisting of zinc, cadmium, mercury, arsenic, antimony, gallium, thallium, bismuth, palladium, ruthenium, osmium and indium, the steps which comprise adjusting the solution pH to lie within the range pH 4 to pH 5, then adjusting the iron and copper content of the solution to lie within the range of 0.1 to 10.0 grams per liter each of iron and copper, treating the solution with an excess of hydrogen sulfide under a pressure between about 15 and 100 pounds per square inch gauge, separating a precipitate containing copper sulfide and other impurities, then adjusting the solution pH to lie between pH 5 and pH 6, passing atmospheric air into and through the resulting solution whereby iron and other impurities are precipitated and remaining hydrogen sulfide stripped off, then removing and discarding the resulting precipitate to yield a purified cobalt solution.

RUTH E. CHURCHWARD,  
FRANCIS K. SHELTON.

## REFERENCES CITED

The following references are of record in the file of this patent:

## UNITED STATES PATENTS

Number Name Date  
2,356,183 Shepard et al. Aug. 22, 1944

## FOREIGN PATENTS

Number Country Date  
298,301 Great Britain Oct. 11, 1928  
543,887 Great Britain Mar. 18, 1942

## OTHER REFERENCES

50 "Handbook of Chemistry and Physics," 16th edition, page 524, Chemical Rubber Publishing Co., Cleveland, Ohio (1931).